

## [54] PHOTOGRAPHIC LIGHT SENSITIVE MATERIAL CONTAINING COPOLYMER LAYER

[75] Inventors: Fumihiko Nishio; Daijiro Nishio; Syu Watarai; Kinji Ohkubo; Yosuke Nakajima, Minami-Ashigara Machi, Japan

[73] Assignee: Fuji Photo Film Co., Ltd., Minami-Ashigara-shi, Kanagawa, Japan

[22] Filed: Sept. 30, 1971

[21] Appl. No.: 188,701

## Related U.S. Application Data

[63] Continuation-in-part of Ser. No. 554,048, May 31, 1966, abandoned.

## [30] Foreign Application Priority Data

June 1, 1965 Japan ..... 40/32032

[52] U.S. Cl. .... 96/85, 96/87 R, 96/114

[51] Int. Cl. .... G03c 1/04, G03c 1/88

[58] Field of Search ..... 96/114, 85, 94, 87 R

## [56] References Cited

## UNITED STATES PATENTS

|           |         |                 |       |        |
|-----------|---------|-----------------|-------|--------|
| 3,408,199 | 10/1968 | Saleck          | ..... | 96/114 |
| 3,341,332 | 9/1967  | Nakajima et al. | ..... | 96/107 |
| 3,360,373 | 12/1967 | Schaller        | ..... | 96/114 |

Primary Examiner—Ronald H. Smith  
Attorney—Sughrue, Rothwell, Mion, Zinn & Macpeak

[57]

## ABSTRACT

A light-sensitive photographic material having at least one layer containing a copolymer represented by the general formula:



wherein  $\text{R}_1$  and  $\text{R}_3$  can be H or  $\text{CH}_3$ ,  $\text{R}_2$  can be an alkyl group having one to three carbon atoms,  $x$  and  $y$  represent positive integers, and  $Z$  represents one of:



where  $n$  is 1-3, exhibits reduced curling upon exposure to moisture.

11 Claims, 6 Drawing Figures

PATENTED JAN 30 1973

3,713,829



FIG.1

FIG.2a



CURL VALUE = 10  
(NO CURL)

FIG.2b



0 < CURL VALUE < 10

FIG.2c



0 < CURL VALUE < 10



CURL VALUE = 0

FIG.2d



CURL VALUE IS  
NEGATIVE

FIG.2e

# PHOTOGRAPHIC LIGHT SENSITIVE MATERIAL CONTAINING COPOLYMER LAYER

## CROSS REFERENCES TO RELATED APPLICATIONS

This application is a continuation in part of application Ser. No. 554,048, filed May 31, 1966, now abandoned, claiming the priority of Japanese Patent Application No. 32,032/1965, filed June 1, 1965.

## BACKGROUND OF THE INVENTION

### 1. Field of the Invention

The present invention relates to a photographic silver halide gelatino light-sensitive material containing a copolymer of N-alkoxymethylalkenoylamide, which illustrates improved curling.

### 2. Description of the Prior Art

It is known that in the production of a photographic silver halide light-sensitive emulsion, a naturally occurring or synthetic high molecular compound other than gelatin, such as, poly-N-vinyl lactams, dextrin, laminarine, mannan, hydroxyethylated cellulose, and the like, increases the covering power of the emulsion (the value of the optical density of the developed emulsion per 1 sq. dm. divided by the gram number of developed silver per 1 sq. dm.). Accordingly, the contrast, the maximum density, etc., can be increased. For example, see U.S. Pat. Nos. 3,003,878 and 3,058,826; French Patent 1,261,846; and Belgian Patents 611,622 and 611,623.

However, as illustrated in FIG. 1 of the accompanying drawing, the sensitivity at the foot portion of the characteristic curve B of the emulsion containing the high molecular weight compound is substantially increased as compared with that of the characteristic curve of the emulsion containing no high molecular weight compound.

Further, it is known that in the production of a photographic silver halide light-sensitive element curling is reduced by adding to the silver halide emulsion thereof naturally occurring or synthetic high molecular weight compounds other than gelatin. For example, polyvinyl alcohol and a copolymer of methylvinyl ether and maleic anhydride or a copolymer of styrene and an acrylic ester may be added. Moreover, it is known that the curling of a photographic light-sensitive element can be reduced by adding a naturally occurring or synthetic high molecular weight compound other than gelatin, such as polyvinyl acetate and a copolymer of butyl acrylate and acrylonitrile, to the undercoating layer. (See French Patent 1,308,399 and German Patent 1,081,755).

The primary object of this invention is to provide a photographic light-sensitive element having low curling characteristics.

Subsidiary objects of this invention are to provide a photographic light-sensitive silver halide emulsion having improved sensitivity, maximum density, and contrast.

These and other objects of the invention will become apparent from the following specification and drawing in which:

## BRIEF DESCRIPTION OF THE DRAWINGS

FIG. 1 is a graph illustrating the improved characteristics obtained with my invention.

FIG. 2 is a schematic representation of various curling values.

## SUMMARY OF THE INVENTION

The inventors have found that the sensitivity of a photographic gelatino silver halide emulsion which has been sensitized to the optimum sensitivity with any standard chemical sensitizer, such as an unstable sulfur compound, a reducing agent, a gold compound, and the like, can be further increased by incorporating in the emulsion certain copolymers of N-alkoxymethyl-alkenoylamide. Further, as shown by curve C of the graph in FIG. 1, not only are the covering power, contrast, and maximum density increased, but also the sensitivity at the foot portion in the characteristic curve is increased, which indicates the addition of the above compound is a very profitable sensitization.

Furthermore, it has been found that the light sensitive element comprising the emulsion layer containing the above compound has a reduced curling tendency.

## DETAILED DESCRIPTION OF THE PREFERRED EMBODIMENTS

The copolymers containing N-alkoxymethylalkenoylamide of the present invention are shown by the following general formula:



wherein  $R_1$  and  $R_3$  are H or  $CH_3$ ;  $R_2$  is an alkyl group having one to three carbon atoms;  $x$  and  $y$  are positive integers; and  $Z$  is one of the following:



wherein  $n$  is 1, 2, or 3, preferably 2.

In a preferred embodiment of the invention  $x$  is from about 1 to about 50, with  $y$  being determined by  $100 - x$ .

It is preferred that the proportion of N-alkoxymethyl-alkenoylamide be above 30 mol percent.

In this invention, the copolymers may be used singly or as mixtures thereof. If the polymerization degree of the copolymer is too high, the compatibility thereof with gelatin will be reduced, and hence it is desirable that the intrinsic viscosity of the copolymer in methanol be less than about 2.0° at 35°C.

Any desired amount of the copolymer may be incorporated in the emulsion in this invention, but the optimum amount thereof for increasing the sensitivity, gamma value and the maximum density is influenced by the type of photographic silver halide emulsion to be adopted, as well as the use to be made of the product. The proportion of the copolymer containing N-alkoxymethylalkenoylamide may be 3-40 percent by weight;

preferably, 2-20 percent by weight, based on the weight of the whole medium in the photographic gelatino silver halide emulsion used (emulsion and copolymer). Good results may also be obtained by adding the copolymer of N-alkoxymethylalkenoylamide in a layer adjacent a gelatino silver halide photographic emulsion layer, and in this case, a suitable proportion of the copolymer is 10-40 percent by weight based on the layer weight.

The optimum proportion of the copolymer for reducing the curling tendency of a photographic light-sensitive element containing the copolymer is influenced by the kind of support and the thickness of coating, but is generally 3-50 percent by weight. Preferably, 10-30 percent by weight based on the whole medium of a photographic gelatino silver halide emulsion layer and/or a subsidiary layer (protection layer, intermediate layer, back layer, etc.) is used.

The copolymer may be added in the emulsion at any time, but is most suitably added after the second ripening, and before coating. The copolymer may be added in the emulsion as a powder, but it is convenient to add it as a 10-20 percent aqueous solution thereof.

The present invention is applicable to any kind of silver halide emulsions, such as a silver iodo-bromide emulsion, a silver chloro-bromide emulsion, and the like. The emulsion may be sensitized preliminary with a sulfur and/or a gold compound, and may contain an optical sensitizer, a polyalkyleneoxide type sensitizer, various stabilizers, a hardening agent, a coating aid, a coupler, etc.

The following are examples of the synthesis of the monomer and the copolymer; however, the invention is not limited to these examples.

### SYNTHESIS 1

#### Synthesis of N-Methoxymethylacrylamide

A mixture of 303 g. (3 mols.) of N-methylolacrylamide, 1,500 ml. of methanol, and 10 ml. of concentrated hydrochloric acid was heated to 45°-50°C., and, while stirring, the N-methylolacrylamide was dissolved slowly to provide a transparent solution. After continuing the reaction for 4 hours at the recited temperature, the solution was neutralized with the addition of anhydrous sodium carbonate. After cooling, the salts formed were removed by filtration, and the excess methanol was removed from the filtrate by distillation under reduced pressure. After the addition of a small amount of hydroquinone as a polymerization inhibitor, the filtrate was subjected to vacuum distillation to provide 290 g. (yield 84 percent) of a colorless liquid having a boiling point of 93°-95°C./1mm.Hg.

Elementary analysis as  $C_5H_9O_2N$ : Calculated N 12.17%; Found N 11.93%

### SYNTHESIS 2

#### Synthesis of N-Ethoxymethylacrylamide

By the same procedure as in Synthesis 1 using a mixture of 303 g. (3 mols) of N-methylolacrylamide, 1,500 ml. of ethanol, and 10 ml. of concentrated hydrochloric acid, 330 g. (yield 85 percent) of a colorless liquid having a boiling point of 103°-104°C./1mm.Hg was obtained. When the liquid was cooled, a colorless crystal (m. p. 21°C.) was formed.

Elementary analysis as  $C_6H_{11}O_2N$ : Calculated N 10.85%; Found N 10.55%.

### SYNTHESIS 3

#### Synthesis of N-Isopropoxymethylacrylamide

By the same procedure as in Synthesis 1 using a mixture of 303 g. (3 mols) of N-methylolacrylamide, 1500 ml. of isopropanol, and 10 ml. of concentrated hydrochloric acid, 351 g. (yield 82 percent) of a colorless liquid having a boiling point of 107°-108°C./2mm. Hg was obtained.

Elementary analysis as  $C_7H_{13}O_2N$ : calculated N 9.78%; Found N 10.25%

### SYNTHESIS 4

#### Synthesis of N-Methoxymethylmethacrylamide

By the same procedure as in Synthesis 1 using a mixture of 115 g. (1 mol) of N-methylolmethacrylamide, 500 ml. of methanol and 3.5 ml. of concentrated hydrochloric acid, 103 g. (yield 80 percent) of a colorless liquid having a boiling point of 83°-85°C./1 mm. Hg was obtained.

Elementary analysis as  $C_6H_{11}O_2N$ : Calculated N 10.85%; Found N 10.80%.

### SYNTHESIS 5

#### Synthesis of N-Ethoxymethylmethacrylamide

By the same procedure as in Synthesis 1 using a mixture of 115 g. (1 mol) of N-methylolmethacrylamide, 500 ml. of ethanol and 3.5 ml. of concentrated hydrochloric acid, 111 g. (yield 78 percent) of a colorless liquid having a boiling point of 104°-105°C./2 mm. Hg was obtained.

Elementary analysis as  $C_7H_{13}O_2N$ : Calculated N 9.78%; Found N 9.83%

### SYNTHESIS 6

#### Synthesis of N-n-Propoxymethylmethacrylamide

By the same procedure as in Synthesis 1, using a mixture of 115 g. (1 mol) of N-methylolmethacrylicamide, 500 ml. of n-propanol and 3.5 ml. of concentrated hydrochloric acid, 120 g. (yield 72 percent) of a colorless liquid having a boiling point of 108°-113°C./1mm. Hg was obtained.

Elementary analysis as  $C_8H_{15}O_2N$ : Calculated N 8.38%; Found N 8.71%

### SYNTHESIS 7

#### Copolymerization of N-Ethoxymethylacrylamide With Other Vinyl Monomers

Copolymerizations of N-ethoxymethylacrylamide with other vinyl monomers in various monomer ratios were carried out under the conditions shown in Table 1 below. When the polymerization was carried out in an aqueous phase, polymer separation was conducted by dialyzing the polymer solution with a cellophane diaphragm and subjecting the dialized polymer to freeze drying. When the polymerization was carried out in an organic solvent, the polymer was precipitated by pouring the polymer solution into a large excess of hexane or ether.

TABLE I

| Example number | M <sub>1</sub> * (g.) | M <sub>2</sub> (g.)  | (A)  | (B) | Polymerization solvent            | (D) (wt. percent) | Polymerization initiator                                                             | (E) °C. | (F) min. | (G) g. | (H) percent | (J) [η] |
|----------------|-----------------------|----------------------|------|-----|-----------------------------------|-------------------|--------------------------------------------------------------------------------------|---------|----------|--------|-------------|---------|
|                |                       |                      |      |     |                                   |                   |                                                                                      |         |          |        |             |         |
| 1.....         | 33.3                  | N-vinyl pyrrolidone. | 66.7 | 3/7 | Aqueous 35% isopropanol solution. | 20                | 2.0 ml. of 30% H <sub>2</sub> O <sub>2</sub> solution and 0.5 g. of L-ascorbic acid. | 40      | 300      | 73     | 73          | 0.280   |
| 2.....         | 53.7                  | do.....              | 46.3 | 5/5 | do.....                           | 20                | do.....                                                                              | 40      | 300      | 87     | 87          | 0.425   |
| 3.....         | 73.0                  | do.....              | 27.0 | 7/3 | do.....                           | 20                | do.....                                                                              | 40      | 300      | 92     | 92          | 0.555   |
| 4.....         | 28.2                  | Acryloyl morpholine. | 71.8 | 3/7 | do.....                           | 20                | do.....                                                                              | 40      | 240      | 83     | 83          | 0.455   |
| 5.....         | 52.2                  | do.....              | 47.8 | 5/5 | do.....                           | 20                | do.....                                                                              | 40      | 240      | 92     | 92          | 0.340   |
| 6.....         | 68.1                  | do.....              | 31.9 | 7/3 | do.....                           | 20                | do.....                                                                              | 40      | 240      | 90     | 90          | 0.280   |

NOTE: (M<sub>1</sub>) N-ethoxymethyl acrylamide, (A) amount of charged monomers, (B) monomer molar ratio, (D) monomer concentration (weight percent), (E) reaction temperature, (F) reaction period, (G) amount of formed polymer (g.), (H) polymerization conversion (weight percent), (J) intrinsic viscosity [η] in methanol at 35.0° C. ([η]).

Polymerization conversion shows following formula:

$$\frac{\text{weight of formed polymer}}{\text{weight of charged monomer}} \times 100 \text{ (percent)} = \frac{G}{M_1 + M_2} \times 100 \text{ (percent)}$$

### EXAMPLE 1

A gelatino silver iodo-bromide emulsion for a high-sensitive X-ray photographic material containing 480 g. of gelatin and 3.3 mols of silver halide consisting of 1.5 mols of silver iodide and 98.5 mol percent of silver bromide, which had already been ripened to the optimum sensitivity by a sulfur sensitizer and a gold-sensitizer, was divided into 11 equal parts and each part of the thus divided emulsion was mixed with 60 ml. of a 10 percent aqueous solution of each of

- a. inactive gelatin,
- b. the polymer obtained in Synthesis 7, Experiment No. 1,
- c. the polymer obtained in Synthesis 7, Experiment No. 2,
- d. the polymer obtained in Synthesis 7, Experiment No. 3,
- e. the polymer obtained in Synthesis 7, Experiment No. 6.

After adding to each of the emulsions 20 ml. of a 1 percent aqueous solution of 4-hydroxyl-6-methyl-1, 3, 3a; 7-tetrazindene as a stabilizer, 8 ml. of a 2 percent acetone-aqueous alkali solution of 2, 4-dichloro-6-oxy-s-triazine as a hardening agent, and 2 ml. of a 4 percent aqueous solution of saponin as a coating aid, the emulsion was applied on a film based on cellulose triacetate to provide a coating of the same thickness and dried. The photographic light-sensitive film was then exposed for one-twentieth sec. in an actinometer having a blue filter and then developed for 4 min. at 20°C. in a developing solution having the following composition:

|                                 |          |
|---------------------------------|----------|
| N-Methyl-p-aminophenol sulfate  | 4g.      |
| Sodium sulfite (anhydrous)      | 60g.     |
| Sodium carbonate (mono-hydrate) | 53g.     |
| Potassium bromide               | 3g.      |
| Hydroquinone                    | 10g.     |
| Water to make                   | 1 liter. |

The photographic densities of the thus developed photographic films are shown in Table II.

TABLE II

|   | Relative sensitivity giving density 0.1 on fog | Relative sensitivity giving density of 1.0 on Fog | Gamma | Fog  |
|---|------------------------------------------------|---------------------------------------------------|-------|------|
| a | 100                                            | 100                                               | 2.23  | 0.05 |
| b | 105                                            | 115                                               | 2.55  | 0.05 |
| c | 107                                            | 115                                               | 2.51  | 0.04 |
| d | 102                                            | 110                                               | 2.47  | 0.05 |
| e | 105                                            | 115                                               | 2.74  | 0.05 |

### EXAMPLE 2

A silver iodo-bromide emulsion which was the same as in Example 1 was mixed with a copolymer ([η] = \*0.20) (\*[η] = intrinsic viscosity in methanol at 35.0°C.) of N-ethoxymethyl acrylamide (50 mol percent) and vinylpyrrolidone (50 mol percent) in various proportions and the same procedure as in Example 1 was repeated using the thus prepared emulsions. The increases in sensitivity are shown in Table III. In these cases, an inactive gelatin was added such that the ratio of the silver halide to the medium was constant.

TABLE III

| Amount of the Copolymer Per 0.3 Mol of Silver Halide (g.) | Relative Sensitivity Giving Density of 1.0 on Fog |     |
|-----------------------------------------------------------|---------------------------------------------------|-----|
|                                                           | 0                                                 | 100 |
| 1.5                                                       | 105                                               |     |
| 3.0                                                       | 112                                               |     |
| 6.0                                                       | 120                                               |     |
| 12.0                                                      | 141                                               |     |

### EXAMPLE 3

Into 100 g. of a gelatino silver chloride emulsion (the weight ratio of gelatin/silver chloride was 4.5/1) for printing papers was added 50 ml. of a 5 percent aqueous solution of the copolymer of this invention and after the addition of a stabilizer, a coating aid, and a hardening agent, the mixture was applied to a photographic paper of 85 g. and dried to provide the dried coating of same thickness in each case.

For comparison, an emulsion containing no polymer of this invention was prepared and applied to a photographic paper by the same conditions to provide a control photographic printing paper.

These light-sensitive elements were allowed to stand for 100 minutes at a temperature of 30°C. and at a humidity of 30% RH and then curling was measured, the results of which are shown in Table IV.

TABLE IV

| No. copolymer                                                                  | Curling Value |     |
|--------------------------------------------------------------------------------|---------------|-----|
|                                                                                | 2.0           | 3.2 |
| Copolymer of N-ethoxymethylacrylamide (70 mol%) and vinylpyrrolidone (30 mol%) |               |     |
| Copolymer of N-ethoxymethylacrylamide (30 mol%) and vinylpyrrolidone (70 mol%) |               | 4.6 |
| Copolymer of N-ethoxymethylacrylamide                                          |               |     |

(70 mol%) and N-morpholinomethylamide (30 mol%)

4.4

## EXAMPLE 4

The purpose of this example was to establish the superiority of the copolymers of the present invention over somewhat similar compounds which are per se known to the prior art, as shown in U.S. Pat. Nos. 3,360,373 Schaller, 3,341,332 Nakajima and 10 3,408,199 Saleck.

## Preparation of the Samples

A 5 percent aqueous solution of each of the following compounds (I-VII) was prepared. To 100 g of a silver chloride emulsion (weight ratio of AgCl to 15 gelatin of 0.84:4; of Ag to gelatin 0.64:4) was added 25 cc of the above-mentioned solution.

The resulting emulsion/solution was coated onto a paper base (document paper used for quick copying; weight 85 g/m<sup>2</sup>) to an Ag amount of 27  $\mu$ g/cm<sup>2</sup>. (i.e. the 20 coating thickness) and the base was dried. The same base was used with each copolymer. This base was cut into a disc having a 10 cm diameter, and the curling value was measured.

The method of determination of the curling value 25 was as follows:

Cut a disc off from the specimen. The diameter of the disc is 10.0 cm. Punch out a hole in the center of the disc. Fix the center hole of the disc on the top of a bar, which, in turn, is fixed to support. Leave the bar 30 with the specimen disc on its tip in a low humidity atmosphere.

After several hours, the disc curls. The curling value is defined as the minimum distance between peripheries on the opposite sides of the curled disc. 35

When the disc does not curl, the distance between peripheries on the opposite sides is the disc. The curling value is thus 10.0 (FIG. 2a).

As the disc begins to curl, one pair of peripheries on the opposite sides gets nearer and nearer. The curling 40 value thus becomes smaller. (FIGS. 2b and 2c).

If the disc continues to curl, a pair of peripheries on the opposite sides contact each other, whereby the curling value is 0.0. (FIG. 2d).

If the disc goes on to curl still more, a pair of peripheries on the opposite side of the curled disc overlap each other. The curling value becomes negative in value. 45 (FIG. 2e).

For the curling determinations, curling was measured after the discs were cut from the specimens (dried at 50°C for 72 hours) and exposed to 30 percent relative humidity at 20°C for 24 hours.

## Compound I: Schaller Pat. (U.S.P. 3,360,373)



## Compound II: Nakajima Pat. (U.S.P. 3,341,332)



Compound III: This invention



Compound IV: This invention



Compound V: This invention



Compound VI: Saleck Pat. (U.S.P. 3,408,199) polymethacrylamide-N-methylol methylether



Compound VII: Saleck Pat. (U.S.P. 3,408,199) polymethacrylamide-N-methylol ethylether



For the gelatin sample, gelatin prepared in the same manner as above was used.

| Compound No. | polymerization ratio | curling value |
|--------------|----------------------|---------------|
| I            | m:n = 1:1            | 6.8           |
| II           | n = 1                | 7.5           |
| III          | x:y = 1:1            | 9.0           |
| IV           | x:y = 1:1            | 8.0           |
| V            | x:y = 1:1            | 8.5           |
| VI           | n = 1                | -3.5          |
| VII          | n = 1                | 3.0           |
| gelatin      | -                    | 6.0           |

55 From the data above, where all conditions were equal but the copolymer used, it can be seen that all copolymers in accordance with the present invention provide superior curling (higher positive values), with the order of descending preference being: Compound III; V; IV. It can also be seen that Compounds VI and VII are inferior to the use of gelatin above.

The following claims are to describe the spirit and scope of the present invention, and are not to be taken as limited to the specific examples heretofore set forth.

60 65 What is claimed is:

1. A light-sensitive photographic material illustrating a reduced curling tendency comprising a support, at least one photographic silver halide emulsion layer and at least one subsidiary layer, at least one of said emulsion layer and subsidiary layer containing one member

selected from the group consisting of the copolymer represented by the general formula,



wherein  $R_1$  and  $R_3$  each represents a member selected from the group consisting of H and  $\text{CH}_3$ ,  $R_2$  represents an alkyl group having one to three carbon atoms,  $x$  and  $y$  represent positive integers, and  $Z$  represents a 15 member selected from the group consisting of



wherein  $n$  is 1 to 3.

2. The photographic light-sensitive material according to claim 1, wherein said support comprises a film.

3. The photographic light-sensitive material according to claim 1, wherein said support comprises a paper.

4. The photographic light-sensitive material according to claim 1, wherein the intrinsic viscosity of said copolymer in methanol at  $35^\circ\text{C}$ . is less than 2.0.

5. The photographic light-sensitive material according to claim 1 wherein the layer containing said copolymer is a silver halide emulsion layer and wherein the proportion of the copolymer is 3-50 percent by weight, based on the whole medium in said silver halide emulsion layer.

6. The photographic element of claim 5 where the proportion is 10-30 percent.

7. The photographic light-sensitive material according to claim 1 wherein the layer containing said copolymer is a subsidiary layer and the proportion of the copolymer is 3-50 percent by weight based on the whole medium of the subsidiary layer.

8. The photographic element of claim 7 where the proportion is 10-30 percent.

10 9. The photographic light-sensitive material according to claim 1 wherein  $Z$  is



10. The photographic light-sensitive material according to claim 1 wherein  $Z$  is

20



25

11. The photographic light-sensitive material according to claim 1 wherein  $Z$  is

30



35

\* \* \* \* \*

45

50

55

60

65